

## UNITED STATES PATENT OFFICE

2,159,466

## REVERSAL DEVELOPMENT OF LIGHT-SENSITIVE SILVER HALIDE EMULSIONS

Gustav Wilmanns, Wolfen, Kreis Bitterfeld, Wilhelm Schneider, Dessau, and Richard Kethur, Bitterfeld, Germany, assignors, by mesne assignments, to Agfa Ansco Corporation, Binghamton, N. Y., a corporation of Delaware

No Drawing. Application October 29, 1937, Serial No. 171,702. In Germany November 10, 1936

2 Claims. (CL 95—88)

Our present invention relates to reversal development of light sensitive silver halide emulsions.

It is known that the reversal development of light-sensitive silver halide emulsion layers may be carried out without intermediate exposure to light if the negative silver image is removed in the second development by means of an alkaline developer containing a small proportion of an odorless sulfur compound, especially thiosinamine. It has also been proposed to use this sulfur compound not in the developing bath but in an intermediate bath or in a clearing bath containing sulfite. These baths containing the sulfur compound have, however, certain disadvantages. In consequence of the instability of the sulfur compounds, for example thiourea derivatives, abundant quantities of silver sulfide separate in the bath whether it be neutral or alkaline. The silver sulfide produces, particularly in the colloid form, brown tints and is not bleached by the usual reducer such as mercuric chloride or potassium ferricyanide used for the purpose. The reversal development with the aid of sulfur compounds in neutral or alkaline solution is in particular little suitable for use in making multi-color pictures because in consequence of the strong blackening of the picture by the separation of black silver sulfide no useful result can be attained.

It is an object of the present invention to avoid or minimize these difficulties and disadvantages of the hitherto known reversal process.

A further object is to provide a photographic reversal process using an intermediate bath with an odorless sulfur compound while preventing precipitation of silver sulfide.

A further object is the provision of a process for developing multi-color pictures according to the reversal method in which process the undesirable blackening of the color tint of the multi-color pictures is avoided.

Further objects will be apparent from the detailed specification following hereafter.

We have discovered that by using the sulfur compound in acid solution the decomposition of the sulfur compounds is quantitatively avoided so that the disturbing precipitation of silver sulfide is prevented and also the blackening of the color tint of the multi-color picture. These acid baths have further the great advantage of a much longer duration than the hitherto known neutral or alkaline baths. The nature of the acid used is without importance, its pH-value being alone decisive. The sulfur compound may be used, for

example, in a solution of acetic acid, oxalic acid, citric acid, sulfuric acid or phosphoric acid.

Suitable odorless sulfur compounds for producing silver sulfide nuclei are, for example, thiourea and its derivatives, for instance N-allyl thiourea (thiosinamine), N, N-diethyl-N'-allyl thiourea, N-phenyl thiourea, N, N-diethanol-N'-phenyl thiourea.

The process is suitable for the reversal development of any black-and-white or color picture, especially for producing color reversal pictures which are produced by color forming development. These latter are first developed in an ordinary negative developer, then treated in an acid bath containing a sulfur compound, which is odorless and can produce silver nuclei, and then developed in a color developer to produce a positive. Silver halide emulsion layers containing dyestuff components which are fast to diffusion such as are described in U. S. patent applications Ser. No. 72,718, filed April 4, 1936; Ser. No. 90,726, filed July 15, 1936; Ser. No. 94,340, filed August 5, 1936; Ser. No. 158,860, filed August 13, 1937; Ser. No. 159,518, filed August 17, 1937; and the U. S. Patent applications Ser. No. 164,499, filed September 18, 1937; and Ser. No. 166,832, filed October 1, 1937, may be developed by the process herein described.

The following example illustrates the invention:

A multi-layer photographic material in which the layers contain dyestuff components fast to diffusion is developed after exposure in one of the usual negative developers for example that known under the registered trade-marks "Amidol" or "Metol", and is then treated with an intermediate bath consisting of 1000 cc. of water, 5 cc. of glacial acetic acid and 0.4 gram of thiosinamine. It is then developed with a color developer, for instance N, N-diethyl-para-phenylene diamine, washed and the silver image removed with Farmer's Reducer, followed by further washing.

What we claim is:

1. In a process of developing a photographic silver halide emulsion by the reversal method, the improvement which comprises interposing between the first and the second development an acid aqueous intermediate bath containing a thiourea capable of forming silver nuclei within said emulsion.

2. A process of producing photographs in color which comprises exposing to light controlled by an object to be reproduced a light-sensitive photographic element comprising a support and a

plurality of silver halide emulsion layers, each layer containing a color former fast to diffusion, developing said photographic element by means of a developer incapable of forming a dye with said color formers, treating said photographic element in an acid aqueous bath containing a thiourea capable of forming silver nuclei in said

emulsion layers, developing said emulsion layers with a developer capable of forming a dyestuff image associated with a silver image, and removing the residual silver from all the layers.

**GUSTAV WILMANNS.**  
**WILHELM SCHNEIDER.**  
**RICHARD KETHUR.**